# EUROPEAN PATENT APPLICATION

(11) **EP 4 628 621 A2**
(43) Date of publication of application: **08.10.2025**
(21) Application number: 25197585.0
(22) Date of filing: 03.12.2021
(51) Int. Cl.: C23C 2/40

(54) **COATED STEEL SHEET AND HIGH STRENGTH PRESS HARDENED STEEL PART AND METHOD OF MANUFACTURING THE SAME**

(30) Priority: 16.12.2020 WO PCT/IB2020/062045
(62) Divisional of application: 21819985.9
(71) Applicant: ArcelorMittal, 1160 Luxembourg (LU)
(72) Inventor: PHILIPPOT, Clément, 57365 Ennery (FR); LE GUILLARD, Sandra, 54800 Mars La Tour (FR); DUSSAUSSOIS, David, 54310 Homecourt (FR); SALIB, Matthieu, 57283 Maizieres-Les- Metz Cedex (FR)
(74) Representative: Lavoix

(57) **Abstract**

The invention deals with a coated steel sheet and press hardened steel part having a composition comprising, by weight percent: C 0.26-0.40%, Mn 0.5-1.8%, Si 0.1-1.25%, Al 0.01-0.1 %, Cr 0.1-1.0%, Ti 0.01-0.1 %, B 0.001-0.004%, P ≤ 0.020%, S ≤ 0.010%, N ≤ 0.010% the remainder of the composition being iron and unavoidable impurities resulting from the smelting. The press hardened steel part comprises a bulk having a microstructure comprising, in surface fraction, more than 95% of martensite and less than 5% of bainite, a coating layer at the surface of the steel part, a ferritic interdiffusion layer between the coating layer and the bulk, and a ratio between the ferritic grain width in the interdiffusion layer GWᵢₙₜ over prior austenite grain size in the bulk PAGS_{bulk}, satisfying following equation (GWᵢₙₜ / PAGS_{bulk})-1 ≥ 30%.

## Description

The present invention relates to coated steel sheets and to high strength press hardened steel parts having good bendability properties.

High strength press-hardened parts can be used as structural elements in automotive vehicles for anti-intrusion or energy absorption functions.
In such type of applications, it is desirable to produce steel parts that combine high mechanical strength, high impact resistance and good corrosion resistance. Moreover, one of major challenges in the automotive industry is to decrease the weight of vehicles in order to improve their fuel efficiency in view of the global environmental conservation, without neglecting the safety requirements.

This weight reduction can be achieved in particular thanks to the use of steel parts with a martensitic or bainitic/martensitic microstructure.

The publication WO2016104881 relates to a hot press forming part used as a structural part of a vehicle or the like, requiring impact resistance characteristics, and more particularly, having a tensile strength of 1300 MPa or greater and a method for manufacturing the same by heating a steel material to a temperature at which an austenite single phase may be formed, and quenching and hot forming thereof using a mold. To obtain such properties, the base steel sheet comprises a thin ferrite layer lower than 50 µm at the surface, and the carbides size and density should be controlled. This ferrite layer in the substrate allow to inhibit the propagation of the fine cracks formed on the plating layer to the base but leads to a low bendability with bending angle lower than 70°.

The publication WO2018179839 relates to a hot-pressed part obtained by hot pressing a steel sheet having a microstructure changing in the thickness direction, with a soft layer made of at least 90% of ferrite, a transition layer made of ferrite and martensite and a hard layer mainly martensitic and has both high strength and high bendability. To obtain such properties, the cold rolled steel sheet is annealed in an atmosphere with a dew point temperature comprises from 50°C to 90°C, which could be harmful to aluminium alloy coating. Further prior art is described in US2017/260599A1 and WO2018/220540A1.

The purpose of the invention therefore is to solve the above-mentioned problem and to provide a press hardened steel part having a combination of high mechanical properties with the tensile strength TS above or equal to 1500 MPa and bending angle higher than 70°. Preferably, the press hardened steel part according to the invention has yield strength YS above or equal to 1250 MPa.

Another purpose of the invention is to obtain a coated steel sheet that can be transformed by hot forming into such a press hardened steel part.

The object of the present invention is achieved by providing a steel sheet according to claim 1. Another object is achieved by providing the method according to claim 2. Another object of the present invention is achieved by providing a press hardened steel part according to claim 3. The steel part can also comprise characteristics of anyone of claim 4. Another object is achieved by providing the method according to claim 5.

The invention will now be described in detail and illustrated by examples without introducing limitations, with reference to the appended figures:
- Figure 1a illustrates a schematic section of the coated steel sheet of trial 4, which is not according to the invention
- Figure 1b represents a schematic section of the press hardened steel part from trial 4 which is not according to the invention
- Figure 2a illustrates a schematic section of the coated steel sheet of trial 3, which is not according to the invention
- Figure 2b represents a schematic section of the press hardened steel part from trial 3 which is not according to the invention
- Figure 3a illustrates a schematic section of the coated steel sheet of trial 2, which is according to the invention
- Figure 3b represents a schematic section of the press hardened steel part from trial 2 which is according to the invention
- Figure 4a illustrates a schematic section of the coated steel sheet of trial 1, which is according to the invention
- Figure 4b represents a schematic section of the press hardened steel part from trial 1 which is according to the invention
- Figure 5a illustrates a schematic section of the coated steel sheet of trial 5, which is not according to the invention
- Figure 5b represents a schematic section of the press hardened steel part from trial 5 which is not according to the invention

The composition of the steel according to the invention will now be described, the content being expressed in weight percent.

According to the invention the carbon content is comprised from 0.26% to 0.40 % to ensure a satisfactory strength. Above 0.40% of carbon, weldability and bendability of the steel sheet may be reduced. If the carbon content is lower than 0.26%, the tensile strength will not reach the targeted value.

The manganese content is comprised from 0.5% to 1.8 %. Above 1.8% of addition, the risk of central segregation increases to the detriment of the bendability. Below 0.5% the hardenability of the steel sheet is reduced. Preferably the manganese content is comprised from 0.5% to 1.3%.

According to the invention, silicon content is comprised from 0.1% to 1.25%. Silicon is an element participating in the hardening in solid solution. Silicon is added to limit carbides formation. Above 1.25%, silicon oxides form at the surface, which impairs the coatability of the steel. Moreover, the weldability of the steel sheet may be reduced. Preferably, the silicon content is from 0.2% to 1.25%. More preferably the silicon content is from 0.3% to 1.25%. More preferably, the silicon content is from 0.3% to 1%.

The aluminium content is comprised from 0.01% and 0.1% as it is a very effective element for deoxidizing the steel in the liquid phase during elaboration. Aluminium can protect boron if titanium content is not enough. The aluminium content is lower than 0.1% to avoid oxidation problems and ferrite formation during press hardening. Preferably the aluminium content is comprised from 0.01% to 0.05%.

According to the invention, the chromium content is comprised from 0.1% to 1.0 %. Chromium is an element participating in the hardening in solid solution and must be higher than 0.1%. The chromium content is below 1.0% to limit processability issues and cost.

The titanium content is comprised from 0.01% to 0.1% in order to protect boron from formation of BN. Titanium content is limited to 0.1% to avoid TiN formation.

According to the invention, the boron content is comprised from 0.001% to 0.004%. Boron improves the hardenability of the steel. The boron content is not higher than 0.004% to avoid a risk of breaking the slab during continuous casting.

Some elements can optionally be added.
Nickel may be added as an optional element up to 0.5% as it can substantially reduce the sensitivity to delayed fracture.

Molybdenum content can optionally be added up to 0.40%. As boron, molybdenum improves the hardenability of the steel. Molybdenum is not higher than 0.40% to limit cost.

According to the invention, niobium can optionally be added up to 0.08% to improve ductility of the steel. Above 0.08% of addition, the risk of formation of NbC or Nb(C,N) carbides increases to the detriment of the bendability. Preferably the niobium content is below or equal to 0.05%.

Calcium may be also added as an optional element up to 0.1%. Addition of Ca at the liquid stage makes it possible to create fine oxides which promote castability of continuous casting.

The remainder of the composition of the steel is iron and impurities resulting from the smelting. In this respect, P, S and N at least are considered as residual elements which are unavoidable impurities. Their content is less than 0.010 % for S, less than 0.020 % for P and less than 0.010 % for N.

The microstructure of the coated steel sheet according to the invention will now be described.

A section of a coated steel sheet of the invention is schematically represented on Fig 3a and Fig 4a. The coated steel sheet comprises a bulk (2) topped by a decarburized layer (3) comprising in upper part a ferrite layer having a thickness from 1µm to 100 µm (4), and a coating layer (1). Preferably, the thickness of the ferrite layer is comprised from 20 µm to 100 µm. More preferably, the thickness of the ferrite layer is from 25 µm to 100 µm. More preferably the thickness of the ferrite layer is from 30 µm to 80 µm.

The bulk of the coated steel sheet (2) has a microstructure comprising, in surface fraction, from 60% to 90% of ferrite, the rest being martensite-austenite islands, pearlite or bainite.

This ferrite is formed during the intercritical annealing of the cold rolled steel sheet. The rest of the microstructure is austenite at the end of the soaking, which transform into martensite-austenite islands, pearlite or bainite during the cooling of the steel sheet.

The decarburized layer present on top of the bulk is obtained during the annealing of the cold rolled steel sheet thanks to the control of the atmosphere in the furnace to set a dew point temperature strictly higher than -10°C and below or equal to 20°C.

The coated steel sheet according to the invention can be produced by any appropriate manufacturing method and the man skilled in the art can define one. It is however preferred to use the method according to the invention comprising the following steps:
A semi-product able to be further hot-rolled, is provided with the steel composition described above. The semi product is reheated at a temperature comprised from 1150°C to 1300°C.

The steel sheet is then hot rolled at a finish hot rolling temperature comprised from 800°C to 950°C.

The hot-rolled steel is then cooled and coiled at a temperature T_{coil} lower than 670°C, and optionally pickled to remove oxidation.

The coiled steel sheet is then optionally cold rolled to obtain a cold rolled steel sheet. The cold-rolling reduction ratio is preferably comprised from 20% to 80%. Below 20%, the recrystallization during subsequent heat-treatment is not favored, which may impair the ductility of the steel sheet. Above 80%, there is a risk of edge cracking during cold-rolling.

The steel sheet is then annealed in an HNx atmosphere with from 0% to 15% of H2, to an annealing temperature T_{A} comprised from 700°C to 850°C and maintained at said annealing temperature T_{A} for a holding time t_{A} comprised from 10s to 1200s, in order to obtain an annealed steel sheet.. Below 700°C, the kinetic of formation of the decarburized layer is too slow to obtain a ferrite layer in its upper part. The holding time t_{A} is above or equal to 10 s to allow the ferrite layer to form, and below or equal to 1200s in order to limit the thickness of this ferrite layer.

During this annealing, the atmosphere in the furnace is controlled to have a dew point temperature T_{DP1} strictly higher than -10°C and below or equal to +20°C in order to form a decarburized layer according to the invention. If T_{DP1} is below or equal to -10°C, the formation of the decarburized layer is slowed down and the ferrite layer is not formed in its upper part. The bendability of the steel part will be too low. If T_{DP1} is higher than 20°C, the surface of the steel sheet may be completely oxidized, impairing coatability and mechanical properties of the sheet
In an embodiment of the invention the annealed steel sheet is heated to an annealing temperature T2 comprised from 700°C to 850°C and maintained at said temperature T2 for a holding time t2 comprised from 10s to 1200s, the atmosphere having a dew point T_{DP2} strictly higher than -10°C and below or equal to +20°C. The steel sheet is then coated with an aluminium alloy coating.

The microstructure of the press hardened steel part according to the invention will now be described. A section of the press hardened steel part is schematically represented on Fig 3b and Fig 4b.

The steel part comprises successively from the bulk to the surface of the steel part:
- a bulk (7) having a microstructure comprising, in surface fraction, more than 95% of martensite and less than 5% of bainite,
- a ferritic interdiffusion layer (6),
- a coating layer (5) based on aluminium.

During the heating of the steel blank cut out of the steel sheet according to the invention, all microstructural elements of the bulk are transformed into austenite, and the ferrite of the decarburized layer is transformed into austenite with wider grain size than the austenite of the bulk. After hot forming, the steel part is then die-quenched. The interdiffusion layer grows from the former wide grain size austenite layer, thus having larger grain width than prior austenitic grain size in the bulk. The ratio between the ferritic grain width in the interdiffusion layer GWᵢₙₜ over prior austenite grain size in the bulk PAGS_{bulk}, satisfies following equation:$\left({GW}_{int} / {PAGS}_{bulk}\right) -1 \times 30 %$ in order to improve bendability of the steel sheet, without deteriorating mechanical properties.
The ferritic grain width is the average distance between two parallel grain boundaries of the interdiffusion layer, grain boundaries being oriented in the direction of the thickness of the sheet. The combination of annealing temperature T_{A}, annealing time t_{A} and dew point temperature T_{DP1} according to the invention promotes the formation of large grain width GWᵢₙₜ in the interdiffusion layer. Moreover, the thermal treatment of the steel blank before the press forming, rules the austenitic grain growth and so the PAGS in the bulk.

In an embodiment, the press hardened steel part may further comprise a martensite layer with a carbon gradient between the bulk and the interdiffusion layer, as represented by (8) in Fig 4b. During the heating of the steel blank, carbon diffuses from the bulk to the surface. The ferrite upper part of the decarburized layer is then transformed in a layer of austenite with a gradient of carbon. During the die-quenching, this layer of austenite with a gradient of carbon is transformed in a layer of martensite with a carbon gradient.

The press hardened steel part according to the invention has a tensile strength TS above or equal to 1500 MPa and a bending angle higher than 70°. The bending angle has been determined on press hardened parts according to the method VDA238-100 bending Standard (with normalizing to a thickness of 1.5 mm).

In a preferred embodiment of the invention, the yield strength YS is above or equal to 1250 MPa. TS and YS are measured according to ISO standard ISO 6892-1.

The press hardened steel part according to the invention can be produced by any appropriate manufacturing method and the man skilled in the art can define one. It is however preferred to use the method according to the invention comprising the following steps:
A coated steel sheet according to the invention is cut to a predetermined shape to obtain a steel blank. The steel blank is then heated to a temperature comprised from 880°C to 950°C during 10s to 900s to obtain a heated steel blank. The heated blank is then transferred to a forming press before being hot formed and die-quenched.

The invention will be now illustrated by the following examples, which are by no way limitative.

### Example

6 grades, which compositions are gathered in table 1, were cast in semi-products and processed into steel sheets, then steel parts, following the process parameters gathered in table 2.

### Table 1 - Compositions

The tested compositions are gathered in the following table wherein the element contents are expressed in weight percent.

| Steel | C | Mn | Si | Al | Cr | Ti | B | P | S | N | Ni | Mo | Nb |
|---|---|---|---|---|---|---|---|---|---|---|---|---|---|
| A | 0.34 | 0.6 | 0.56 | 0.043 | 0.32 | 0.017 | 0.002 | 0.009 | 0.0018 | 0.0027 | 0.43 | 0.19 | 0.052 |
| B | 0.32 | 0.7 | 0.35 | 0.03 | 0.5 | 0.026 | 0.002 | 0.014 | 0.0022 | 0.0059 | 0.028 | 0.21 | - |
| C | 0.36 | 0.6 | 0.53 | 0.035 | 0.34 | 0.014 | 0.003 | 0.011 | 0.001 | 0.0034 | 0.4 | 0.20 | 0.049 |
| D | 0.33 | 0.6 | 0.53 | 0.028 | 0.33 | 0.013 | 0.003 | 0.013 | 0.001 | 0.0041 | 0.4 | 0.17 | 0.046 |
| E | 0.36 | 1.3 | 0.28 | 0.003 | 0.25 | 0.02 | 0.003 | 0.01 | 0.002 | 0.006 | - | - | - |
| F | 0.21 | 1.2 | 0.27 | 0.018 | 0.15 | 0.037 | 0.002 | 0.01 | 0.002 | 0.006 | 0.012 | - | - |

Steels A-D are according to the invention.

Underlined values: not corresponding to the invention

### Table 2 - Process parameters

Steel semi-products, as cast, were reheated at 1200 °C, hot rolled with a finish hot rolling temperature comprised from 800 to 950°C, coiled at 550°C and cold rolled with a reduction rate of 60%. Steel sheets are then heated to a temperature T_{A} and maintained at said temperature for a holding time t_{A}, in an HNx atmosphere with 5% of H₂, having a controlled dew point. The steel sheets were then cooled down to a temperature from 560 to 700°C and then hot dip coated with an aluminium-silicon coating comprising 10% of silicon.

Samples 1,2,5 and 6 did undergo a second annealing at a temperature T₂ before coating, the steel sheet being maintained at said T₂ temperature for a holding time t₂, in an HNx atmosphere with 5% of H₂ and a controlled dew point. The following specific conditions were applied:

| Trial | Steel | Soaking | | | Second soaking | | |
|---|---|---|---|---|---|---|---|
| | | t_{A} (s) | T_{A} (°C) | T_{DP1} (°C) | t₂ (s) | T₂ (°C) | T_{DP2} (°C) |
| 1 | A | 135 | 850 | 10 | 70 | 800 | 0 |
| 2 | B | 135 | 850 | 10 | 70 | 800 | 0 |
| 3 | C | 240 | 755 | -10 | - | - | - |
| 4 | D | 30 | 730 | -40 | - | - | - |
| 5 | E | 10800 | 700 | 0 | 70 | 750 | 0 |
| 6 | F | 135 | 850 | 10 | 70 | 800 | 0 |

Underlined values: not corresponding to the invention

The coated steel sheets were analyzed, and the corresponding properties of decarburized layer are gathered in table 3.

**Table 3 - Properties of the decarburized layer of the coated steel sheet**

| Trial | Presence of decarburized layer | Thickness of the ferrite upper part of the decarburized layer (µm) |
|---|---|---|
| 1 | yes | 60 |
| 2 | yes | 35 |
| 3 | yes | - |
| 4 | no | - |
| 5 | yes | 140 |
| 6 | yes | 60 |

Underlined values: not corresponding to the invention

The coated steel sheets were then cut to obtain a steel blank, heated at 900°C during 6 minutes and hot-formed. The steel parts were analyzed and the corresponding microstructure, ferritic grain width in interdiffusion layer GWᵢₙₜ, and prior austenite grain size in the bulk PAGS_{bulk} are gathered in table 4. Mechanical properties are gathered in Table 5.

**Table 4 - Microstructure of the press hardened steel part**

| Trial | Bulk microstructure | (GWᵢₙₜ / PAGS_{bulk} )-1 | GWᵢₙₜ (µm) | PAGS_{bulk} (µm) |
|---|---|---|---|---|
| 1 | 100% martensite | 83% | 9.9 | 5.4 |
| 2 | 100% martensite | 128% | 16.9 | 7.4 |
| 3 | 100% martensite | 27% | 6.6 | 5.2 |
| 4 | 100% martensite | -2% | 4.9 | 5 |
| 5 | 10% ferrite | | | |
| | 70% bainite | | | |
| | 20% martensite | n.d | 8.3 | n.d |
| 6 | 100% martensite | 45% | 8.9 | 7.8 |

Underlined values: not corresponding to the invention

n.d: non determined

The surface fractions, ferritic grain width in the interdiffusion layer and PAGS are determined through the following method: a specimen is cut from the press hardened steel part, polished and etched with a reagent known per se, to reveal the microstructure. The section is afterwards examined through optical or scanning electron microscope, for example with a Scanning Electron Microscope with a Field Emission Gun ("FEG-SEM") at a magnification greater than 5000x, coupled to a BSE (Back Scattered Electron) device.

### Table 5 - Mechanical properties of the press hardened steel part

Mechanical properties of the tested samples were determined and gathered in the following table:

| Trial | TS (MPa) | Bending angle at 1.5mm (°) | YS (MPa) |
|---|---|---|---|
| 1 | 1691 | 77 | 1361 |
| 2 | 1649 | 73 | 1296 |
| 3 | 1922 | 36 | 1488 |
| 4 | 1917 | 42 | 1527 |
| 5 | 1566 | 34 | 1183 |
| 6 | 1410 | 65 | 1060 |

Underlined values: do not match the targeted values

The examples show that the steel parts according to the invention, namely examples 1-2 are the only one to show all the targeted properties thanks to their specific compositions and microstructures.

Figure 3a represents a schematic section of the coated steel sheet of trial 2. The combination of process parameters of the invention, annealing temperature T_{A}, annealing time t_{A} and dew point temperature T_{DP1} allow to obtain a decarburized layer (3), in which a layer of ferrite is formed in the upper part (4).

The coated steel sheet is then hot formed. Fig 3b represents a schematic section of the press hardened steel part of trial 2.

The grain width of ferrite formed in the interdiffusion layer (5) is a heritage of the pure ferrite layer in which austenite formation takes place during heating, with larger grain size. The interdiffusion layer grows on this large austenite grain size. The grain width of ferrite in the interdiffusion layer (6) is then larger than prior austenite grain size in the bulk (7), leading to good bendability with bending angle higher than 70°.
Figure 4a represents a schematic section of the coated steel sheet of trial 1. The combination of process parameters of the invention, annealing temperature T_{A}, annealing time t_{A} and dew point temperature T_{DP1} allow to obtain a decarburized layer (3), in which a layer of ferrite is formed in the upper part (4), thicker than in trial 1 due to the higher C content.

The coated steel sheet is then hot formed. Fig 4b represents a schematic section of the press hardened steel part of trial 1.

The grain width of ferrite formed in the interdiffusion layer (6) is a heritage of the pure ferrite layer in which austenite formation takes place during heating, with larger grain size. The interdiffusion layer grows on this large austenite grain size . The grain width of ferrite in the interdiffusion layer (6) is then larger than prior austenite grain size in the bulk (7), leading to good bendability with bending angle higher than 70°. Moreover, due to the thick ferrite layer (4) in the coated steel sheet, a layer of martensite with a carbon gradient is formed between the bulk and the interdiffusion layer in the press hardened steel part, leading to tensile strength higher than 1500 MPa.

In trial 3, the coated steel sheet has a decarburized layer, without ferrite layer in its upper part, as represented schematically in Fig 2a. The absence of ferrite layer is due to the low dew point temperature T_{DP1} of -10°C, which slow down the kinetics of the decarburization.

The coated steel sheet is then hot formed. Figure 2b represents a schematic section of the press hardened steel part from trial 3. Due to the absence of the ferrite layer, the ferritic grain width in the interdiffusion layer (6) is then equivalent to prior austenite grain size in the bulk (7), leading to a low bending angle below 70°.

In trial 4, the low dew point temperature T_{DP1} of -40°C implies an absence of the decarburized layer and ferrite layer in the coated steel sheet.

Fig 1a represents a schematic section of the coated steel sheet of this trial, with the coating layer (1) and the bulk (2).

The coated steel sheet is then hot formed. Figure 1b represents a schematic section of the press hardened steel part from trial 4. Due to the absence of the ferrite layer, the ferritic grain width in the interdiffusion layer (6) is then equivalent to prior austenite grain size in the bulk (7), leading to a low bending angle below 70°.

In trial 5, the steel sheet is maintained during 10800s at soaking temperature, which form in the coated steel sheet, a thicker ferrite layer in the decarburized layer than previous trials. Fig 5a represents a schematic section of the coated steel sheet of trial 5, with the coating layer (1) the decarburized layer (3), the thicker ferrite layer (4) with coarser grain size, and the bulk (2).

The coated steel sheet is then hot formed and Fig 5b represents a schematic section of the press hardened steel part from trial 5. During the heating of the steel part, the microstructure of the bulk is austenitic, and the thick ferrite layer is transformed in a layer of austenite with gradient of carbon. But due to the thickness of the ferrite layer higher than 100 µm, a layer of ferrite remains present between the interdiffusion layer and the layer of austenite with gradient of carbon.

During die quenching of the steel part, the ferrite layer is still present and the layer of austenite with carbon gradient transforms into a martensite layer with gradient of carbon, leading to a multi-phased layer. This triggers a decrease of yield strength.

In trial 6, the steel sheet has a low carbon level of 0.21%. This low carbon content combined to the process parameters, leads to a decarburized layer in the coated steel sheet with the ferrite layer. Nevertheless, the yield strength and tensile strength of the press hardened steel part are not achieved because of the low level of carbon.

## Claims

1. A coated steel sheet made of a steel having a composition comprising, by mass percent:
C : 0.26 - 0.40 %
Mn : 0.5 - 1.8 %
Si: 0.2- 1.25 %
Al : 0.01 - 0.1 %
Cr : 0.1 - 1.0 %
Ti: 0.01 - 0.1 %
B: 0.001 - 0.004 % $P \leq 0.020 %$ $S \leq 0.010 %$ $N \leq 0.010 %$
and comprising optionally one or more of the following elements, by mass percent: $Ni \leq 0.5 %$ $Mo \leq 0.40 %$ $Nb \leq 0.08 %$ $Ca \leq 0.1 %$
the remainder of the composition being iron and unavoidable impurities resulting from the smelting,
said coated steel sheet comprising from the bulk to the surface of the coated steel sheet:
- a bulk with a microstructure comprising, in surface fraction, from 60% to 90% of ferrite, the rest being martensite-austenite islands, pearlite or bainite,
- such bulk being topped by a decarburized layer comprising in upper part a ferrite layer having a thickness from 1µm to 100 µm
- a coating layer made of aluminum or aluminium alloy.

2. A method for producing a coated steel sheet according to claim 1, said method comprising the following successive steps:
- casting a steel to obtain a slab, said steel having a composition according to claim 1,
- reheating the slab at a temperature Tᵣₑₕₑₐₜ comprised from 1100°C to 1300°C,
- hot rolling the reheated slab at a finish hot rolling temperature comprised from 800°C to 950°C
- coiling the hot rolled steel sheet at a coiling temperature T_{coil} lower than 670°C to obtain a coiled steel sheet,
- optionally pickling the coiled steel sheet,
- cold rolling the coiled steel sheet to obtain a cold rolled steel sheet
- Heating the hot rolled steel sheet or the cold rolled steel sheet to an annealing temperature T_{A} comprised from 700°C to 850°C and maintaining the steel sheet at said temperature T_{A} for a holding time t_{A} comprised from 10s to 1200s, to obtain an annealed steel sheet, the atmosphere comprising from 0% to 15% of H2 and having a dew point T_{DP1} strictly higher than -10°C and below or equal to +20°C
- cooling said annealed steel sheet to a temperature range from 560°C to 700°C,
- Coating the annealed steel sheet with aluminium or with an aluminium alloy coating
- Cooling the coated steel sheet to room temperature to obtain a steel sheet having a microstructure according to claim 1.

3. A press hardened steel part, the steel part having a composition comprising, by mass percent:
C : 0.26 - 0.40 %
Mn : 0.5 - 1.8 %
Si: 0.2 - 1.25 %
Al : 0.01 - 0.1 %
Cr : 0.1 - 1.0 %
Ti: 0.01-0.1 %
B: 0.001 - 0.004 % $P \leq 0.020 %$ $S \leq 0.010 %$ $N \leq 0.010 %$
and comprising optionally one or more of the following elements, by mass percent: $\begin{matrix}Ni \leq 0.5 % \\ Mo \leq 0.40 %\end{matrix}$ $Nb \leq 0.08 %$ $Ca \leq 0.1 %$
the remainder of the composition being iron and unavoidable impurities resulting from the smelting,
said steel part comprising successively from the bulk to the surface of the steel part:
- a bulk having a microstructure comprising, in surface fraction, more than 95% of martensite and less than 5% of bainite,
- a ferritic interdiffusion layer,
- a coating layer based on aluminium,
wherein the ratio between the ferritic grain width in said interdiffusion layer GWᵢₙₜ over prior austenite grain size in the bulk PAGS_{bulk}, satisfies the following equation: $\left({GW}_{int}/{PAGS}_{bulk}\right) - 1 \geq 0.3$
And having a tensile strength TS above or equal to 1500 MPa, a yield strength YS above or equal to 1250 MPa and a bending angle higher than 70°, TS and YS being measured according to ISO standard ISO 6892-1, and the bending angle according to the method VDA238-100 bending Standard (with normalizing to a thickness of 1.5 mm).

4. A press hardened steel part according to claim 3, wherein the press hardened steel part comprises a layer of martensite with a carbon gradient between said bulk and said ferritic interdiffusion layer.

5. A process for manufacturing a press hardened steel part according to anyone of claims 3 to 4, comprising the following successive steps:
- providing a steel sheet said steel having a composition according to claim 1, or produced by a method according to claim 2,
- cutting said steel sheet to a predetermined shape, so as to obtain a steel blank,
- heating the steel blank to a temperature comprised from 880°C to 950°C during 10s to 900s to obtain a heated steel blank,
- transferring the heated blank to a forming press,
- hot-forming the heated blank in the forming press to obtain a formed part,
- die-quenching the formed part
